

Patented Feb. 12, 1929.

1,701,799

## UNITED STATES PATENT OFFICE.

RUDOLPH E. SINRAM AND CLYDE T. HELLER, OF LONG ISLAND CITY, NEW YORK.

### CAULKING POWDER.

No Drawing. Application filed March 25, 1925, Serial No. 18,365. Renewed December 29, 1928.

Among the principal objects which the present invention has in view are: to provide a composition which makes a steam-tight joint between threaded members; to avoid rusting or corroding of the threaded members; and to provide a compound of the character mentioned which will not "freeze" or otherwise adhere to the threaded members.

10 The compound referred to consists of 15 portions by volume of (domestic) flour of any ordinary household variety; one portion by volume of sal-ammoniac; and one portion by measure of pulverized iron. 15 These materials are thoroughly mixed and packed as a powder in suitably sealed containers.

Just prior to using, the powder is mixed in cold water to the consistency of a paste.

20 The paste is then spread on the externally threaded member of a screw joint, and the two threaded members are then screwed one upon the other, in the same manner as when using articles such as white or red lead.

It will be found that the joint thus filled 25 is steam, air, and water-tight, and that it will remain thus for an indefinite period, and as far as now known, the joint may be freely opened by retracting the threaded members when it will be found that the 30 metal has not been corroded or adhered to the caulking composition.

We claim:

1. A caulking powder comprising a domestic flour substance; sal-ammoniac; and 35 pulverized iron in proportions substantially as herein described.

2. A caulking powder comprising approximately 15 portions of domestic flour by volume; approximately one portion of sal-ammoniac by volume; and approximately one portion of pulverized iron by volume, said portions being thoroughly mixed while dry.

RUDOLPH E. SINRAM.  
CLYDE T. HELLER.